

## UNITED STATES PATENT OFFICE

2,232,745

## METALLURGY OF IRON

Marvin J. Udy, Niagara Falls, N. Y.

No Drawing. Application January 28, 1939,  
Serial No 253,440

15 Claims. (Cl. 75—27)

This invention relates to metallurgy and has for an object the provision of improved metallurgical processes and materials. An important object of the invention is to provide an improved method of altering the compositions of metal products containing iron. Another important object of the invention is to provide improved exothermic mixtures suitable for use in the production of metallic iron. A more specific object of the invention is to provide a novel method of producing metallic iron products suitable for use in the production of high-strength castings from metal, of the type commonly produced in foundry cupolas, which is suitable for use in the production of relatively low-strength castings.

The invention will be described hereinafter more particularly with respect to its use in the production of metal suitable for use in the production of high-strength castings, but it is to be understood that certain features are useful in general metallurgical procedures involving the production of metallic iron.

In the production of metallic iron products suitable for use in the production of high-strength castings, the invention employs the principle of dilution of relatively impure metallic iron products with relatively pure metallic iron to form resulting products containing metallic iron in increased proportions and, consequently, containing other components in proportions smaller than in the relatively impure products subjected to treatment. In accordance with the invention, dilution is effected by reacting in contact with the impure metallic products, while molten, exothermic mixtures capable of reacting to produce relatively pure molten iron.

In many foundries, operations are confined for the most part to the production of metallic iron products suitable for use in the production of ordinary soft iron, or low-strength, castings, products containing for example, about 3.15 percent carbon and about 2.25 percent silicon. Iron products suitable for use in producing relatively high-strength castings (products containing, for example, about 2.9 percent carbon and about 2.0 percent silicon) require careful control of the production processes or special equipment for their production. The average small foundry is not provided with the special equipment or the necessary technical supervisory facilities to produce such products, and consequently, the output of such a foundry is limited to products which can be pro-

duced by means of simple operations of the type of cupola operations.

The present invention permits the operations of foundries to be made more flexible by enabling ordinary foundry operators to modify or alter, conveniently and accurately, the composition of all or any part of the material produced in any furnace heat without the necessity for employing special equipment. The invention provides exothermic mixtures capable of producing relatively pure metallic iron in definite quantities per unit of weight, and, by means of simple calculations, a foundry operator may determine the proper quantity required to effect dilution of ordinary soft iron to the extent desired to form a product containing iron, carbon and silicon in desired proportions. Cupolas may be operated as usual to produce the customary soft iron product, and dilution can be effected by addition of the exothermic mixtures to the ladles commonly employed for receiving molten metal from the cupolas.

The exothermic mixtures of the invention may consist essentially of iron oxide, lime (CaO) and a silicon-containing reducing agent, preferably low-carbon ferrosilicon. The iron oxide employed may be in the form of iron oxide ores containing the usual impurities of such ores, or a relatively pure iron oxide product such, for example, as mill scale or pyrites cinders may be employed. In forming the exothermic mixtures, I prefer to employ ferric oxide ( $Fe_2O_3$ ) or a material containing ferric oxide as the source of iron oxide, but an oxide containing iron in a lower state of oxidation such, for example, as magnetite ( $Fe_3O_4$ ) may be employed. When an iron oxide product such as magnetite, containing iron in the lower state of oxidation, is employed in an exothermic mixture, an additional substance containing readily available oxygen must be incorporated in the reaction mixture in order to provide for smooth and complete reaction. Magnetite-bearing material such as mill scale may be used advantageously in forming exothermic mixtures also by treating it preliminarily to oxidize the iron to the ferric condition with the production of ferric oxide. Oxidation may be accomplished readily by sintering under oxidizing conditions. When high temperatures are desired, the exothermic mixtures in which the iron oxide is present entirely as ferric oxide may include one or more oxidizing agents capable of reacting with silicon to develop temperatures higher than those developed by reaction of silicon with ferric

oxide ( $Fe_2O_3$ ). Usually, I prefer to incorporate at least small amounts of one or more oxidizing agents of the type of sodium nitrate, sodium chlorate and manganese dioxide in the 5 exothermic mixtures to insure the production of molten reaction products and to increase the temperature of the metal undergoing alteration, as higher temperatures promote the development of greater strength and uniformity in castings. The lime ( $CaO$ ) may be present 10 in the exothermic mixtures in free or uncombined condition, or it may be present in chemical combination with the iron oxide. The exothermic mixtures preferably are 15 formed of components in the form of particles minus 100-mesh in size, and the particles of the components preferably are thoroughly and intimately mixed. Mixing and grinding may be accomplished simultaneously by grinding 20 the components together in suitable apparatus, as, for example, in a ball mill.

I have found that a mixture of lime, ferric 25 oxide, and ferrosilicon when added to a ladle of molten soft iron reacts exothermically to produce pure iron and to dilute the soft iron to any desired carbon and silicon contents, depending upon the relative quantities of soft iron employed and pure iron produced. When fresh lime ( $CaO$ ), ferric oxide and ferrosilicon are mixed intimately 30 in the form of particles minus 100-mesh in size and the mixtures formed into compact masses, they react readily on a ladle of molten iron. Due, however, to the radiation losses, it usually is advisable to increase the heat developed somewhat 35 by the addition of excess silicon and an oxygen carrying agent like sodium nitrate or sodium chloride or manganese dioxide to oxidize the excess silicon and produce additional heat. This is particularly desirable in the treatment of small 40 batches of iron. Large batches do not need as much excess silicon. I have found that for the best results the iron oxide and lime should be chemically combined by heating the two materials in contact at elevated temperatures. The reaction 45 between the iron oxide and the silicon is much more effective and rapid when the lime and iron oxide are chemically combined.

The lime ( $CaO$ ) and ferric oxide may be combined chemically by heating a mixture of the 50 two materials in finely divided form and under non-reducing conditions to a temperature of about 1200° C. or higher. The heating treatment may be so conducted as to result in the production 55 of a fused product, or heating may be so controlled as to effect chemical combination without fusion resulting. When the heating treatment is carried out at a temperature sufficiently high to effect fusion, it is desirable to have present calcium oxide in amount sufficient to combine with 60 all ferric oxide present. Otherwise, some magnetite may be formed with consequent loss in heat developing capacity. When magnetite-bearing material is to be subjected to a sintering treatment under oxidizing conditions, lime may be 65 mixed with the magnetite-bearing material to effect oxidation of the magnetite to ferric oxide and combination of calcium oxide with ferric oxide in a single operation. The lime and ferric oxide employed in forming the exothermic mixtures 70 may be combined chemically in any suitably proportions. Good results may be obtained when the lime and iron oxide are chemically combined in the ratio, one molecule of calcium oxide ( $CaO$ ) to one molecule of ferric oxide ( $Fe_2O_3$ ). 75 I may control the amount of silicon in the final

metal product either by adjusting the amount of lime in the exothermic mixture employed, or by adjusting the amount of silicon relatively to the amount of iron oxide in the exothermic mixture. When silicon control is accomplished through 5 control of the amount of lime employed, I employ an oxidizing agent with excess silicon, the silicon, lime and oxidizing agent being employed in proportions such as to effect oxidation of all silicon and reduction of substantially all iron with 10 the production of a calcium silicate slag containing calcium oxide and silica in a molecular ratio of about 1.0 to  $2CaO:1 SiO_2$  and with the development of sufficient heat to make the slag 15 thinly fluid. Higher ratios of lime to silica may be employed but ratios within the range set forth are quite satisfactory. When silicon control is accomplished by adjusting the amount of silicon relatively to the amount of iron oxide, the adjustment is such that silicon is employed in an 20 amount insufficient to reduce all of the iron oxide present. In this case, a portion of the iron, in oxide form, enters the slag with calcium oxide and silica, forming a slag more readily fusible than a relatively pure calcium silicate slag. 25

In its preferred form, the invention contemplates the production and use of exothermic mixtures containing insufficient silicon to reduce all of the iron oxide, as considerable economy is effected owing to the saving in silicon through 30 the production of readily fusible slags containing iron oxide, the iron oxide retained in the slag being usually no more expensive than lime as a slag-forming material. The proportions of iron oxide and silicon for incorporation in the exothermic mixture may be calculated according to the following equation:



When lime ( $CaO$ ) is present in the mixture in the ratio, one molecule of calcium oxide to one molecule of ferric oxide ( $Fe_2O_3$ ), the slag produced as a result of the reaction will contain calcium oxide, ferrous oxide and silicon dioxide in equi-molecular proportions, and the reaction may be represented roughly by the following equation: 4



While, as hereinbefore pointed out, I prefer to 5 employ ferrosilicon as the reducing agent for reducing iron oxide to produce pure molten iron, my invention also contemplates the use of silicon-containing reducing agents in which the silicon is alloyed with such other metals as nickel, 5 aluminum, magnesium and calcium. Also, those exothermic mixtures of my invention, in which ferric oxide chemically combined with lime is employed, may include such alloys of silicon as chrome silicon and ferrochrome silicon. Such exothermic mixtures are incapable of producing practically pure molten iron, as the molten iron produced will contain chromium; they may be employed for producing iron-chromium alloys directly, upon ignition in suitable containers, or they may be caused to react in contact with molten metals to produce final products of altered compositions. Preferably, the exothermic mixtures of my invention contain no compounds of metals reducible to the metallic state, by exothermic reaction of the mixtures, other than iron oxide, or other than iron oxide and manganese dioxide when the manganese dioxide is used primarily for the purpose of increasing exothermicity.

The following example illustrates a process of

my invention for diluting molten cupola metal with pure molten iron: To 20 pounds of molten cupola iron (analyzing 3.15% C, 2.33% Si, .73% Mn) in a small ladle, I added 11.89 pounds of an intimate mixture consisting of 9.7 pounds of calcium ferrite (analyzing  $\text{Fe}_2\text{O}_3$  69.0%,  $\text{CaO}$  22.1%), .48 pounds of sodium nitrate and 1.71 pounds of ferrosilicon (analyzing 75% Si). The mixture ignited immediately and the reaction was complete 10 in four and one-half (4 1/2) minutes. The slag weighed 7.8 pounds and analyzed as follows:  $\text{FeO}$  26.8%,  $\text{CaO}$  25.4%,  $\text{SiO}_2$  32.60% (balance, sodium compounds from oxidizing agent and magnesium compounds from lime). The metal analyzed as 15 follows: C 2.72%, Si 2.08%, Mn .71%. The tensile strength of the altered iron product was 43,000 pounds per square inch as compared with 39,000 pounds per square inch before treatment.

It will be appreciated that the treatment of 20 the small quantity of metal employed in the above-noted example (20 pounds) involves some difficulties, particularly with respect to temperature control in view of large radiation losses. The results obtained serve to show, however, how the 25 heat of reaction can be used to keep even small amounts of metal hot and at the same time reduce the carbon and silicon contents and produce metal suitable for use in the production of high-strength castings. Obviously, even better 30 results can be obtained in treating larger quantities of metal.

Dilution or alteration of the compositions of 35 metals to any suitable or desired degrees may be carried out. The degree of alteration or dilution to be practiced or achieved is a matter for determination on the basis of economic considerations.

I claim:

1. The method of altering the composition of 40 a metal product containing iron which comprises igniting in contact with the metal product while molten an exothermic mixture consisting essentially of ferric oxide chemically combined with calcium oxide, and a silicon-containing reducing agent.

45 2. The method of altering the composition of a metal product containing iron which comprises igniting in contact with the metal product while molten an exothermic mixture consisting essentially of ferric oxide chemically combined with calcium oxide, and a low-carbon silicon-containing reducing agent.

50 3. The method of altering the composition of a metal product containing iron which comprises igniting in contact with the metal product while molten an exothermic mixture consisting essentially of ferric oxide chemically combined with calcium oxide, and low-carbon ferrosilicon.

55 4. The method of altering the composition of a metal product containing iron which comprises igniting in contact with the metal product while molten an exothermic mixture consisting essentially of ferric oxide chemically combined with calcium oxide, a silicon reducing agent and oxidizing material capable of developing by reaction with silicon a temperature higher than that resulting from reaction of the ferric oxide with silicon.

60 5. An exothermic mixture suitable for use in the production of metallic iron consisting essentially of ferric oxide chemically combined with calcium oxide, and a silicon-containing reducing agent.

65 6. An exothermic mixture suitable for use in the production of metallic iron consisting essentially of ferric oxide chemically combined with

calcium oxide, and a low-carbon silicon-containing reducing agent.

7. An exothermic mixture suitable for use in the production of metallic iron consisting essentially of ferric oxide chemically combined with calcium oxide, and low-carbon ferrosilicon.

8. An exothermic mixture suitable for use in the production of metallic iron consisting essentially of ferric oxide chemically combined with calcium oxide, a silicon-containing reducing agent and oxidizing material capable of developing by reaction with silicon a temperature higher than that resulting from reaction of the ferric oxide with silicon.

9. An exothermic mixture suitable for use in the production of metallic iron consisting essentially of ferric oxide chemically combined with calcium oxide and a silicon-containing reducing agent, the silicon being present in the mixture in an amount sufficient to reduce only a portion 20 of the iron of the ferric oxide to the metallic state, whereby control of silicon in the metal resulting from reaction and the production of a readily fusible iron oxide-bearing slag are provided for.

25 10. An exothermic mixture suitable for use in the production of metallic iron consisting essentially of ferric oxide chemically combined with calcium oxide and a low-carbon silicon-containing reducing agent, the silicon being present in the mixture in an amount sufficient to reduce only a portion 30 of the iron of the ferric oxide to the metallic state, whereby control of the silicon in the metal resulting from reaction and the production of a readily fusible iron oxide-bearing 35 slag are provided for.

11. An exothermic mixture suitable for use in the production of metallic iron consisting essentially of ferric oxide chemically combined with calcium oxide and low-carbon ferrosilicon, the 40 silicon being present in the mixture in an amount sufficient to reduce only a portion of the iron of the ferric oxide to the metallic state, whereby control of silicon in the metal resulting from reaction and the production of a readily fusible iron oxide-bearing 45 slag are provided for.

12. An exothermic mixture suitable for use in the production of metallic iron consisting essentially of ferric oxide chemically combined with calcium oxide, a silicon-containing reducing agent 50 and oxidizing material capable of developing by reaction with silicon a temperature higher than that resulting from reaction of the ferric oxide with silicon, the silicon being present in the mixture in an amount sufficient to reduce only a 55 portion of the iron of the ferric oxide to the metallic state, whereby control of silicon in the metal resulting from reaction and the production of a readily fusible iron oxide-bearing slag are provided for.

60 13. An exothermic mixture suitable for use in the production of a product containing metallic iron and chromium, consisting essentially of ferric oxide chemically combined with calcium oxide, and an alloy containing chromium and silicon.

65 14. An exothermic mixture suitable for use in the production of a product containing metallic iron and chromium, consisting essentially of ferric oxide chemically combined with calcium oxide, and ferrochrome silicon.

70 15. An exothermic reaction mixture suitable for use in the treatment of molten metallic iron consisting essentially of ferric oxide chemically combined with calcium oxide, silicon-containing 75

reducing material and oxidizing material capable of developing by reaction with silicon a temperature higher than that resulting from reaction of the ferric oxide with silicon, the silicon being present in the mixture in an amount insufficient to reduce all of the iron of the ferric oxide to the metallic state and the calcium oxide being pres-

ent in an amount greater than that equivalent to one molecule of calcium oxide per atom of silicon present in the mixture, whereby control of silicon in the molten metal and the production of a readily fusible, basic, iron oxide-bearing slag 5 are provided for.

MARVIN J. UDY.